

Aug. 2, 1927.

**1,637,762**

J. B. CAMPBELL

## FLOOR COVERING

Filed Sept. 7, 1926



INVENTOR.  
John B Campbell  
Allen Allen  
ATTORNEY.

## UNITED STATES PATENT OFFICE.

JOHN B. CAMPBELL, OF SALEM, NEW JERSEY, ASSIGNOR TO THE J. B. CAMPBELL MANUFACTURING COMPANY, OF SALEM, NEW JERSEY, A CORPORATION OF NEW JERSEY.

## FLOOR COVERING.

Application filed September 7, 1926. Serial No. 133,789.

My invention relates to the formation of floor coverings on a base fabric of saturated felt, usually asphalt saturated with a pigmented wear coating, and a suitable fac-  
5 ing on the back.

The present practice in the manufacture of floor coverings is to provide a piece of asphalt saturated felt base, which is given a thin coat of a suitable paint, often a water  
10 paint, or an encaustic paint, but normally a thin oil paint of fairly rapid drying qualities, said paint being applied to the back of the asphalt saturated felt. It has been proposed to add this paint while the asphalt  
15 saturant is still hot, so that it will partly penetrate the felt, due to the shrinkage of the asphalt during the cooling period of the felt saturant.

The only results of such a paint back on  
20 floor coverings of the felt base type is that it gives an appearance which is more satisfactory than the plain black body, and perhaps in some instances, will prevent the asphalt from exuding any sticking to the floor  
25 where the felt base body is in use. I say "in some instances" because the films of paint used are so thin that they will not supply any real service, and their full value  
30 can practically be allocated to their appearance value.

It is the object of my invention to do away with the use of paint as a backing for felt base floor covering, and instead to apply thereto a coating or film of powdered vegetable matter or the like adhesively secured to the back of the sheet and preferably rolled, brushed or calendered to a smooth finish.

As a typical example of my invention, I  
40 may apply to the asphalt saturated felt base, when the saturant is set, an adhesive coating, preferably of quick hardening properties, and quite thin in body so as not to interfere with full flexibility of the final product.

45 Of substances which have been employed in my work as an adhesive, I may refer to cellulose products, hard asphalt in heat liquefied condition, and varnishes with quick driers, having waterproof and chemical  
50 proof character, and certain glues which are adapted to this work.

Referring first to the use of cellulose lac-  
quers, the important element to consider is the effect of the lacquer on the asphalt of the

saturated felt or whatever saturant is used. 55 It should adhere to the asphalt or other saturant without bringing the same up through to the surface of the film.

Thus, as solvents for nitro-cellulose, I will use for applying to asphalt felt not more than 85% of ethyl acetate, and the balance of the solvent will be mainly ethyl alcohol which may be denatured. The cellulose lacquer is applied in usual manner of applying same, and the powdered cork or other matter is brought into contact through a suitable nozzle. A brushing and rolling operation or sanding operation may follow to get the coat quite smooth. It is important in the use of powdered cork, in obtaining the best 70 effects, to use the most finely divided cork that is obtainable, since a better effect can be gained with the most complete adhesion in a thin film of the vegetable matter coating. 75

In using asphalt, an asphalt of high penetration and a quite thin film is used, with the remaining steps the same, since quick hardening, tensile strength, and flexibility are required, and in a thick layer such an asphalt 80 will be brittle.

The powdered cork is much the best material to employ so far as floor covering is concerned, and the degree of adulteration with other vegetable or mineral powders should be kept low, if economy requires any adulteration. 85

In a floor covering the effect of a film or layer of powdered cork applied to the back of a piece of asphalt saturated felt with a 90 waterproof binder is of very high value from a number of points of view. In the first place the adhesive layer imparts strength which is lacking in the asphalt saturated felt base. In the second place, the 95 layer of cork itself adds greatly to the strength. Since the films of adhesive may be and will be of flexible nature, and the cork is finely divided, the flexibility of the finished product will be greater with the cork backing, than if it were omitted, since the tendency of the asphalt in the felt to become stiff and crack is reduced, and the film of adhesive with the insulating layer of cork will keep up the nature of the asphalt for a 100 long period. 105

Thirdly, cork is water resisting in na-  
ture, and together with the binder will re-

sist moisture and retain its qualities during long exposure thereto. Since paint surfaced floor coverings are used largely in places where it is required to wash the floors frequently, and where moisture, grease and the like is expected as a daily occurrence, it is valuable in a floor covering to provide the facing of powdered cork on the underside where moisture is held 10 and does not dry off.

In the fourth place, it is a valuable feature of the cork film that it imparts a non-slipping quality to the rug, due to its softness of feel. This non-slipping quality 15 is especially desirable in rugs but applies to other styles of floor covering in a like manner.

In appearance, the cork backing is very important. It gives a complete concealment of the black asphalt, and gives the 20 appearance of being part of a solid base of cork, whose lasting qualities on the floor is known and has been extolled for a lengthy period in the linoleum industry. It may 25 be applied in suitably dyed colors, or dyed after application, or given a size of cellulose lacquer or other varnish in which color has been incorporated, after it has been applied. In some cases, a colorless lacquer 30 may be added as a size, thus providing a reversible rug in which the cork backing will last a long while as a wear surface.

In using various varnishes and glue adhesives, the requirements of process are not 35 substantially different from the use of the cellulose lacquers, but a quick drying property, permitting an immediate working of the vegetable powder film is important in the adhesive used, as well as its inert nature to 40 solvents and reagents, after it is set.

The finishing of the flooring felt with a 45 painted face or wear surface will not require any difference treatment from the usual floor covering manufacturing processes.

The drawing is a sectional perceptive of a piece of floor covering.

It is a formal showing of the product 50 exaggerated in the layers shown, which layers will be bonded to each other. Thus

the asphalt saturated felt base is indicated in the drawing at 1, to which is applied the wear surface of paint 2, which will be in whatever design desired, and is usually printed onto the base. The back of the felt 55 is faced with a thin layer of adhesive 3, in which is imbedded the cork powdered face 4.

Where other materials are used instead of cork, there will be a consequent decrease in value of the product. Wood flour will give 60 temporarily the appearance of the cork backing, but would have to be well sized in order to last.

The backing differs from the application of sheeted fabric or other material to the 65 flooring, since the particles of cork remain discrete although they cover the whole body, and hence elasticity is not interfered with. In cork also there is but little expansion and contraction or warping tendency which is 70 important in the flooring. A certain amount of elasticity is called for in flooring of this type, because wear along certain paths across the flooring will push outwardly the 75 portions thereof not worn, thus resulting in warping, unless the various elements making up the body are elastic.

Having thus described my invention what I claim as new and desire to secure by Letters Patent is:

1. In combination with the body of a 80 floor covering of felt base type, a backing therefor formed of a thin film of powdered vegetable matter bound to the body by an adhesive.

2. In combination with the body of a 85 floor covering of felt base type, a backing therefor formed of a thin film of powdered cork bound to the body by an adhesive.

3. In combination with the body of a 90 floor covering of felt base type, a backing therefor formed of a thin film of powdered vegetable matter bound to the body by a pyroxylin adhesive.

4. In combination with the body of a 95 floor covering of felt base type, a backing therefor formed of a thin film of powdered cork bound to the body by a pyroxylin adhesive.

JOHN B. CAMPBELL.